# EUROPEAN PATENT SPECIFICATION

(11) **EP 3 476 964 B1**
(45) Date of publication and mention of the grant of the patent: **27.01.2021**
(21) Application number: 17855743.5
(22) Date of filing: 14.09.2017
(51) Int. Cl.: C21D 6/02, C21D 8/02, C21D 8/04, C21D 9/46, C22C 38/06, B65D 41/10, C21D 1/26, C21D 1/28, C22C 38/04, C21D 6/00

(54) **STEEL SHEET FOR CROWN CAPS, PRODUCTION METHOD THEREFOR, AND CROWN CAP**
STAHLBLECH FÜR KRONKORKEN, HERSTELLUNGSVERFAHREN DAFÜR UND KRONKORKEN
TÔLE D'ACIER POUR CAPSULE-COURONNE, PROCÉDÉ DE FABRICATION CORRESPONDANT, ET CAPSULE-COURONNE

(30) Priority: 29.09.2016 JP 2016192247
(43) Date of publication of application: 01.05.2019
(73) Proprietor: JFE Steel Corporation, Tokyo 100-0011 (JP)
(72) Inventor: KARIYA Nobusuke, Tokyo 100-0011 (JP); HIRAGUCHI Tomonari, Tokyo 100-0011 (JP); KOJIMA Katsumi, Tokyo 100-0011 (JP); UMEMOTO Masashi, Tokyo 100-0011 (JP); TSUJIMOTO Masami, Tokyo 100-0011 (JP)
(74) Representative: Haseltine Lake Kempner LLP
(86) International application number: PCT/JP2017/033179
(87) International publication number: WO 2018/061787

(56) References cited:
- EP-A1- 1 291 447
- EP-A1- 2 253 729
- WO-A1-2012/077628
- WO-A1-2016/084353
- CN-A- 102 766 800
- JP-A- H1 072 640
- JP-A- S6 134 159
- JP-A- S50 139 013
- JP-A- 2009 263 788
- JP-A- 2016 079 505

## Description

### Technical Field

The present invention relates to a steel sheet, excellent in shape uniformity and pressure resistance to resist internal pressure, for crown caps used for beer bottles; a method for manufacturing the same; and a crown cap prepared using the steel sheet for crown caps.

### Background Art

Metal stoppers called crown caps are widely used for containers for beverages such as refreshing drinks and alcohols. In general, crown caps are manufactured from a thin steel sheet by press forming and include a disk-shaped portion for covering the mouth of a bottle and a pleated portion placed therearound. The bottle is tightly sealed by crimping the pleated portion to the mouth of the bottle.

Internal pressure is generated in bottles filled with beer or carbonated drinks by contents therein. The crown caps need to have high pressure resistance such that the seal of the bottles is not broken by the deformation of the crown caps and the contents do not leak when the internal pressure increases due to a change in temperature or the like. When steel as material has sufficient strength and is, however, poor in formability, the shapes of pleats are non-uniform; hence, even if a crown cap is crimped to the mouth of a bottle, sufficient airtightness is not obtained in some cases. Therefore, the steel needs to have excellent formability.

A steel sheet used to manufacture crown caps is mainly an SR (single-reduced) steel sheet. This is obtained in such a manner that a steel plate is thinned by cold rolling, followed by annealing and temper rolling. The thickness of a steel sheet for conventional crown caps is generally 0.22 mm or more and sufficient pressure resistance and formability can be ensured by the use of an SR material made of mild steel used for cans for foods and drinks.

In recent years, gauge reduction has been increasingly required for steel sheets for crown caps, as well as steel sheets for cans, for cost reduction purposes. When the thickness of a steel sheet for crown caps is 0.20 mm or less, a crown cap manufactured from a conventional SR material is short of pressure resistance. In order to ensure the pressure resistance, it is conceivable to use a DR (double-reduced) steel sheet which is obtained by performing secondary cold rolling after annealing and which can take advantage of work hardening to compensate for a reduction in strength due to gauge reduction. However, an increase in rolling reduction ratio during secondary cold rolling hardens a steel sheet to reduce the formability thereof. In a process of forming a crown cap, a central portion is drawn to a certain degree in the initial stage of forming and an outside edge portion is then formed into a pleated shape. In the case of a steel sheet with low formability, a shape failure in which shapes of pleats are non-uniform occurs in some cases. A crown cap with a non-uniform pleated shape has a problem that pressure resistance is not obtained by capping a bottle, contents leak, and the crown cap does not play a role as a lid. When the strength of a steel sheet is low, a crown cap may possibly be detached due to insufficient pressure resistance even if the pleated shape thereof is uniform. Furthermore, a method for evaluating pressure resistance has become strict because of the gauge reduction of steel sheets for crown caps. Conventional pressure resistance evaluation has been performed by a method in which a crown cap is crimped to a bottle, air is injected from an upper portion of the crown cap, the internal pressure of the bottle is increased at a constant rate, and the pressure at which the crown cap is detached is measured. In recent years, the following method has been used: a method in which after the internal pressure is increased, a predetermined pressure is held for a certain time and then the internal pressure is further increased.

Hitherto, techniques below have been proposed for the purpose of obtaining a steel sheet excellent in both strength and formability under gauge reduction.

Patent Literature 1 discloses an ultra-thin mild steel sheet with a thickness of 0.4 mm or less, excellent in can strength and can formability, for containers. The ultra-thin mild steel sheet contains N: 0.0040% to 0.0300% and Al: 0.005% to 0.080% on a mass basis, has a 0.2% offset yield strength of 430 MPa or less and a total elongation of 15% to 40% as determined by a tensile test using a JIS No. 5 test specimen, and also has a Q⁻¹ of 0.0010 or more due to internal friction.

Patent Literature 2 discloses a steel sheet for high-strength, high-formability cans. The steel sheet contains C: 0.001% to 0.080%, Si: 0.003% to 0.100%, Mn: 0.10% to 0.80%, P: 0.001% to 0.100%, S: 0.001% to 0.020%, Al: 0.005% to 0.100%, N: 0.0050% to 0.0150%, and B: 0.0002% to 0.0050% on a mass basis and also contains 0.01% to 1.00% of crystal grains having an elongation rate of 5.0 or more in a cross section along the rolling-direction ,in terms of an area fraction.

Patent Literature 3 discloses a steel sheet for cans with high-strength and high-formability. The steel sheet contains C: 0.001% to 0.040%, Si: 0.003% to 0.100%, Mn: 0.10% to 0.80%, P: 0.001% to 0.100%, S: 0.001% to 0.020%, Al: 0.005% to 0.100%, N: more than 0.015% to 0.020%, and B: 0.0002% to 0.0050% on a mass basis, the content of N which is present in the form of AlN being 0.0060% or less; also contains crystal grains having an average grain size of 5.00 µm or more and an elongation rate of 2.50 or less in a cross section along the rolling-direction; and has a tensile strength of 550 MPa or more and a breaking elongation of 7% or more.

EP 2253729 A1 and EP 1291447 A1 disclose cold rolled steel sheets.

### Citation List

### Patent Literature

PTL 1: Japanese Unexamined Patent Application Publication No. 2001-49383
PTL 2: Japanese Unexamined Patent Application Publication No. 2013-28842
PTL 3: Japanese Unexamined Patent Application Publication No. 2012-72439

### Summary of Invention

### Technical Problem

However, there is a problem in that in the case of applying the conventional techniques to the gauge reduction of a steel sheet for crown caps, the performance of a crown cap cannot be ensured by any of them. The steel sheet described in Patent Literature 1 is mild and contains a large amount of N; hence, increasing the secondary cold rolling reduction ratio for the purpose of obtaining necessary strength increases the anisotropy to impair the formability. In addition, in Patent Literature 1, while a two-piece can is evaluated for flange formability and can strength after can-making, the pressure resistance of a crown cap after the crown cap is formed and a bottle is capped with the crown cap is not at all described. Also in the case with the steel sheet described in Patent Literature 2, while the strength of the steel sheet is increased due to N, it is difficult to achieve both pressure resistance and formability required for crown caps. In the steel sheet described in Patent Literature 3, while both the increase in strength of the steel sheet and the formability thereof are achieved by controlling the amount of solute N, the average size of crystal grains, and the elongation rate of the crystal grains, the steel sheet is not suitable for crown cap forming in which drawing is dominant, because can body forming which is different in forming method from crown cap forming and in which bending is dominant is performed.

The present invention has been made in view of the above problems. It is an object of the present invention to provide a steel sheet, having sufficient pressure resistance and formability regardless of gauge reduction, for crown caps; a method for manufacturing the same; and a crown cap. Solution to Problem

The scope of the invention is as defined in the appended claims.

According to the present invention, a steel sheet, having sufficient pressure resistance and formability regardless of gauge reduction, for crown caps; a method for manufacturing the same; and a crown cap can be provided.

### Brief Description of Drawings

[Fig. 1] Fig. 1 is an illustration showing a method for measuring the cross-sectional hardness of a side portion of a crown cap.
[Fig. 2] Fig. 2 is an illustration showing the shapes of pleats of a crown cap.

### Description of Embodiments

A steel sheet for crown caps according to the present invention has a composition containing C: 0.02% to 0.08%, Si: 0.02% or less, Mn: 0.10% to 0.60%, P: 0.020% or less, S: 0.020% or less, Al: 0.01% to 0.06%, and N: 0.0100% to 0.0180% on a mass basis, the remainder being Fe and inevitable impurities, wherein N total-(N as AlN) is 0.0090% to 0.0170%, the maximum grain size of a carbide is 2.0 µm or less in a cross section in a rolling direction, and the yield strength is 420 MPa to 600 MPa in the rolling direction. The steel sheet for crown caps according to the present invention is described below.

First, the composition of the steel sheet for crown caps according to the present invention is described. The unit "%" of the content is all "mass percent".

### (Content of C: 0.02% to 0.08%)

When the content of C is less than 0.02%, the strength of the steel sheet is low, the cross-sectional hardness of a side portion of a crown cap after crown cap forming is low, and the pressure resistance thereof is low. However, when the content of C is greater than 0.08%, the strength of the steel sheet is significantly high and therefore the shapes of pleats of the formed crown cap are non-uniform, leading to shape failures. Furthermore, the maximum grain size of the carbide in the cross section in the rolling direction is large and therefore the shapes of the pleats of the formed crown cap are non-uniform, leading to shape failures, which cause a reduction in pressure resistance. Thus, the content of C is set to 0.02 % to 0.08%. The content of C is preferably 0.03% or more. The content of C is preferably 0.06% or less.

### (Content of Si: 0.02% or less)

Containing a large amount of Si impairs the formability of the crown cap for the same reason as C. Furthermore, the deterioration in surface treatability of the steel sheet and the reduction in corrosion resistance thereof are caused. Therefore, the content of Si is set to 0.02% or less. The lower limit of the content of Si is not particularly limited. Excessively reducing Si causes an increase in steelmaking cost. Therefore, the content of Si is preferably set to 0.004% or more.

### (Content of Mn: 0.10% to 0.60%)

When the content of Mn is less than 0.10%, it is difficult to avoid hot shortness even in the case of reducing the content of S and a problem such as surface cracking occurs during continuous casting. Thus, the content of Mn is set to 0.10% or more. However, containing a large amount of Mn impairs the formability of the crown cap for the same reason as C and Si. Thus, the content of Mn is set to 0.60% or less. In the case where more excellent pressure resistance is required, the content of Mn is preferably 0.20% or more.

### (Content of P: 0.020% or less)

When the content of P is greater than 0.020%, the steel sheet is hard and the reduction in corrosion resistance thereof is caused in addition to the reduction in formability of the crown cap. Thus, the upper limit of the content of P is set to 0.020%.

### (Content of S: 0.020% or less)

S is a harmful element which forms inclusions in the steel sheet to cause the reduction in hot ductility of the steel sheet and the deterioration in corrosion resistance thereof. Thus, the upper limit of the content of S is set to 0.020%.

### (Content of Al: 0.01% to 0.06%)

Al is a necessary element serving as a deoxidizer during steelmaking. When the content of Al is less than 0.01%, deoxidization is insufficient, leading to the increase in amount of inclusions and the deterioration in formability of the crown cap. On the other hand, Al forms AlN with N in steel to reduce the amount of solute N in steel. When the content of Al is greater than 0.06%, the amount of N total-(N as AlN) described below is not sufficiently obtained and the strength of the steel sheet is low. Thus, the content of Al is set to 0.01% to 0.06%. The content of Al is preferably set to 0.01% to 0.04%.

### (Content of N: 0.0100% to 0.0180%)

When the content of N is less than 0.0100%, the amount of N total-(N as AlN) described below is not sufficiently obtained, the strength of the steel sheet is low, and the pressure resistance is low. However, when the content of N is greater than 0.0180%, the strength of the steel sheet is excessively high, leading to the deterioration in formability of the crown cap and the reduction in pressure resistance thereof. Thus, the content of N is set to 0.0100% to 0.0180%. In the case where more excellent pressure resistance is required, the content of N is preferably 0.0135% or more.

### (N total-(N as AlN): 0.0090% to 0.0170%)

In the present invention, in order to ensure the strength, a desired amount of solute N is necessary. In the composition of steel in the present invention, N in the steel is probably mainly present in the form of AlN. Therefore, (N total-(N as AlN)) obtained by subtracting the amount of N present in the form of AlN (N as AlN) from the total amount of N (N total) is regarded as the amount of solute N. When the content of N total-(N as AlN) is less than 0.0090%, the strength of the steel sheet is low and the pressure resistance is low. However, when the content of N total-(N as AlN) is greater than 0.0170%, the strength of the steel sheet is excessively high, the formability of the crown cap is low, and the pressure resistance thereof is low. Thus, the content of N total-(N as AlN) is set to 0.0090% to 0.0170%. The content of N total-(N as AlN) is preferably set to 0.0110% to 0.0170%. Incidentally, the amount of N present in the form of AlN can be confirmed in such a manner that AlN is dissolved and extracted using, for example, a 10% Br-methanol solution and N present in the form of AlN is quantitatively analyzed by absorptiometry.

The remainder are Fe and the inevitable impurities.

Next, the microstructure of the steel sheet for crown caps according to the present invention is described. The steel sheet for crown caps according to the present invention has a microstructure containing the carbide and the maximum grain size of the carbide in the cross section in the rolling direction is 2.0 µm or less. In the steel composition in the present invention, the carbide in the steel is mainly present in the form of cementite. When the maximum grain size of the carbide in the cross section in the rolling direction is greater than 2.0 µm, the shapes of the pleats of the formed crown cap are non-uniform, leading to shape failures, which cause a reduction in pressure resistance. The reason for this is unclear and is considered as described below. A pleated portion of the crown cap is a site suffering tensile and compressive strains or strain superimposed with tension and compression in each of the rolling direction of the steel sheet, directions perpendicular to the rolling direction, and thickness directions. Therefore, it is conceivable that if coarse carbides are present, then strain locally concentrates during forming to cause shape failures. When the maximum grain size of the carbide (cementite) is less than 0.3 µm, the steel sheet has excessively high strength and the formability of the crown cap may possibly be impaired. Therefore, the maximum grain size of cementite is 0.3 µm or more. For the metallographic structure of cementite, a through-thickness cross section parallel to the rolling direction of the steel sheet is polished and is then etched with an etchant (3 volume percent nital), a through-thickness one-fourth position (in the above cross section, a one-fourth position from a surface in a thickness direction) is observed over 10 fields of view at 2,000x magnification using a scanning electron microscope (SEM), and cementite is identified by visual judgment using a microstructure photograph taken with the SEM. For the size of cementite grains, the area of each cementite grain is determined by image analysis and is converted into the equivalent circle diameter, which is defined as the size of the cementite grain. The size of a cementite grain which is largest in size in the 10 fields of view is defined as the maximum grain size of the carbide.

Next, mechanical properties of the steel sheet for crown caps according to the present invention are described. The steel sheet for crown caps according to the present invention is required to have such a pressure resistance that the crown cap is not detached by the internal pressure in a bottle. The thickness of steel sheets conventionally used for crown caps was 0.22 mm or more. In gauge reduction in which the thickness of a sheet is 0.20 mm or less, strength higher than ever is necessary. When the yield strength of the steel sheet in the rolling direction is less than 420 MPa, it is difficult to impart sufficient pressure resistance to such a thinned crown cap as described above. However, when the yield strength thereof is greater than 600 MPa, the compressive stress in the circumferential direction of the pleated portion of the crown cap is high and the yield strength exceeds the critical buckling strength in the initial stage of forming the crown cap; hence, large pleats occur in the pleated portion to cause shape failures. Thus, the yield strength in the rolling direction is set to 420 MPa to 600 MPa. In order to achieve a good crown cap shape and pressure resistance, the yield strength is preferably 450 MPa to 600 MPa. Incidentally, the yield strength can be measured by a metallic material tensile test method specified in "JIS Z 2241". A desired yield strength can be obtained in such a manner that the composition is adjusted; the coiling temperature during hot rolling, the average heating rate after cold rolling, the annealing temperature, and the average cooling rate after annealing are adjusted; and the cooling stop temperature and the retaining temperature after cooling stop are adjusted. A yield strength of 420 MPa to 600 MPa can be obtained in such a manner that the above-mentioned composition is set, the coiling temperature in a hot rolling step is set to 670 °C or less, the average heating rate in a temperature range A from 500 °C to 600 °C in a heating course in a continuous annealing step after a cold rolling step is set to 10 °C/s to 30 °C/s, annealing is performed at an annealing temperature B in a temperature range from 620 °C to 740 °C, cooling is performed from the annealing temperature B to a cooling stop temperature C in a temperature range from 400 °C to 580 °C at an average cooling rate of 20 °C/s or more, the retention time for which retaining is performed in the temperature range from 400 °C to 580 °C after cooling at the above average cooling rate is stopped is set to 30 seconds to 90 seconds, and secondary cold rolling is performed at a rolling reduction ratio of 1.0% to 12%. Incidentally, the yield strength of the steel sheet in a direction (width direction) perpendicular to the rolling direction is preferably 450 MPa to 600 MPa.

The steel sheet for crown caps is punched into a circular blank, which is then formed into the crown cap by press forming. After formation, the crown cap is crimped to the mouth of a bottle with a capper, whereby the airtightness after capping is maintained. When the strength of the side portion after crown cap forming is low, the crown cap is detached from the bottle mouth in some cases when the bottle is held in such a condition that the internal pressure of the bottle is high, leading to the leakage of contents in the bottle. The strength of the side portion after crown cap forming closely correlates with the Vickers hardness of a cross section thereof. When the cross-sectional hardness of the side portion of the crown cap is less than 180 Hv, the strength of the side portion of the crown cap is low, leading to a reduction in airtightness, that is, a reduction in pressure resistance by a pressure test. However, when the cross-sectional hardness of the side portion of the crown cap is greater than 220 Hv, the strength of the side portion of the crown cap is excessively high and therefore cracks occur in the portion. In order to achieve both a good crown cap shape and pressure resistance, the cross-sectional hardness of the side portion of the crown cap is set to 180 Hv to 220 Hv. The cross-sectional hardness of the side portion of the crown cap is preferably 190 Hv to 220 Hv.

The cross-sectional hardness of the side portion of the crown cap can be evaluated by a method specified in "JIS Z 2244". In the present invention, positions for evaluating the cross-sectional hardness of the side portion of the crown cap are in a cross section of the side portion of the crown cap between pleats of the crown cap and a measuring is performed in terms of Vickers hardness. In the present invention, as shown in Fig. 1, the measuring positions are set to five points, in total, including one point at the center, two points in an upper surface direction of the crown cap, and two points in a downward direction of the crown cap, on the center being at a position (H/2) corresponding to half the height H of the crown cap. The Vickers indentation load is set to 100 gf and the intervals between the points are set to 3d (d: the length of a diagonal of an indentation). The average of the Vickers hardness values at the five points is defined as the cross-sectional hardness of the side portion of the crown cap. A desired cross-sectional hardness can be obtained by forming the crown cap from the steel sheet for crown caps, the steel sheet being obtained in such a manner that the composition is adjusted; the coiling temperature during hot rolling, the average heating rate after cold rolling, the annealing temperature, and the average cooling rate after annealing are adjusted; and the secondary cold rolling reduction ratio is adjusted. A cross-sectional hardness of the side portion of the crown cap of 180 Hv to 220 Hv can be obtained by forming the crown cap from the steel sheet for crown caps, the steel sheet being obtained in such a manner that the above-mentioned composition is set, the coiling temperature in the hot rolling step is set to 670 °C or less, the average heating rate in the temperature range A from 500 °C to 600 °C in the heating course in the continuous annealing step after the primary cold rolling step is set to 10 °C/s to 30 °C/s, annealing is performed at the annealing temperature B in the temperature range from 620 °C to 740 °C, cooling is performed from the annealing temperature B to the cooling stop temperature C in the temperature range from 400 °C to 580 °C at an average cooling rate of 20 °C/s or more, the retention time for which holding is performed in the temperature range from 400 °C to 580 °C after cooling at the above average cooling rate is stopped is set to 30 seconds to 90 seconds, and secondary cold rolling is performed at a rolling reduction ratio of 1.0% to 12%.

Next, an example of the method for manufacturing the steel sheet for crown caps according to the present invention is described. The steel sheet for crown caps according to the present invention is manufactured by performing the following steps: a hot rolling step of coiling a steel material (steel slab) having the above-mentioned composition at a temperature of 670 °C or less after finish rolling in hot rolling; a pickling step of performing pickling as required after the hot rolling step; a primary cold rolling step of performing cold rolling after the pickling step; a continuous annealing step of performing heating at an average heating rate of 10 °C/s to 30 °C/s in a temperature range A from 500 °C to 600 °C in a heating course after the primary cold rolling step, annealing at an annealing temperature B in a temperature range from 620 °C to 740 °C, cooling from the annealing temperature B to a cooling stop temperature C in a temperature range from 400 °C to 580 °C at an average cooling rate of 20 °C/s or more, and retaining in the temperature range from 400 °C to 580 °C for a retention time of 30 seconds to 90 seconds after cooling at the above average cooling rate is stopped; and a secondary cold rolling step of performing cold rolling at a rolling reduction ratio of 1.0% to 12% after the continuous annealing step. Incidentally, in descriptions below, the temperature is the surface temperature of the steel sheet or the like. Regarding the average heating rate and the average cooling rate, the values thereof are values obtained by calculation based on the surface temperature. The average heating rate in the temperature range A from 500 °C to 600 °C in the heating course is given by ((600 °C - 500 °C) / heating time from 500 °C to 600 °C). The average cooling rate from the annealing temperature B to the cooling stop temperature C is given by ((annealing temperature B - cooling stop temperature C) / cooling time from annealing temperature B to cooling stop temperature C).

Upon manufacturing the steel sheet for crown caps according to the present invention, molten steel is prepared by a known process using a converter or the like so as to contain the above-mentioned chemical components and is then cast into a slab by, for example, a continuous casting process. Subsequently, the slab is preferably subjected to rough rolling in high heating temperature. A rough rolling process is not particularly limited. In order to ensure that N total-(N as AlN) is 0.0090% or more, the heating temperature of the slab is preferably 1,200 °C or more. In order to further increase N total-(N as AlN), the heating temperature of the slab is preferably 1,230 °C or more.

The finish rolling temperature in the hot rolling step is preferably 850 °C or higher from the viewpoint of the stability of rolling load. However, unnecessarily raising the finish rolling temperature makes it difficult to manufacture a thin steel sheet in some cases. In particular, the finish rolling temperature is preferably within the range of 850 °C to 960 °C.

It is not preferable that the coiling temperature in the hot rolling step is higher than 670 °C, because the amount of AlN precipitated in steel after coiling is increased, the amount of N total-(N as AlN) is less than 0.0090%, and thereby the yield strength of the steel sheet in the rolling direction is less than 420 MPa, and the cross-sectional hardness of the side portion of the crown cap after crown cap forming is less than 180 Hv in some cases. It is not preferable that the coiling temperature in the hot rolling step is higher than 670 °C, because the maximum grain size of the carbide in the cross section in the rolling direction is greater than 2.0 µm, and the shapes of the pleats of the crown cap become non-uniform during crown cap forming, leading to shape failures in some cases. Thus, the coiling temperature in the hot rolling step is set to 670 °C or less. In order to sufficiently ensure the amount of N total-(N as AlN), the coiling temperature in the hot rolling step is preferably 640 °C or less. However, when the coiling temperature is excessively low, the yield strength of the steel sheet in the rolling direction is greater than 600 MPa and the cross-sectional hardness of the side portion of the crown cap after crown cap forming is greater than 220 Hv in some cases. Therefore, the coiling temperature is preferably 500 °C or more.

Subsequently, pickling is performed as required. Pickling may only be capable of removing surface scales and conditions for pickling need not be particularly limited. Alternatively, a process such as mechanical removal may be used instead of pickling.

The rolling reduction ratio in the primary cold rolling step is not particularly limited and is preferably 85% to 94% for the purpose of adjusting the thickness of the steel sheet after secondary cold rolling to 0.20 mm or less.

In the continuous annealing step, heating is performed at an average heating rate of 10 °C/s to 30 °C/s in the temperature range A from 500 °C to 600 °C. It is not preferable that heating is performed at an average heating rate of less than 10 °C/s in the temperature range A, because the precipitation of AlN occurs during heating, the amount of N total-(N as AlN) is less than 0.0090%, the yield strength of the steel sheet in the rolling direction is less than 420 MPa, the cross-sectional hardness of the side portion of the crown cap after crown cap forming is less than 180 Hv, and the pressure resistance is low. Thus, the average heating rate in the temperature range A is set to 10 °C/s or more. The average heating rate therein is preferably set to 12 °C/s or more. In the case of performing heating at an average heating rate of more than 30 °C/s in the temperature range A, the steel sheet is excessively hard, the shape becomes non-uniform in crown cap forming, and the pressure resistance is decreased. Therefore, the average heating rate in the temperature range A is set to 30 °C/s or less. When the average heating rate in the temperature range A is greater than 30 °C/s, problems such as overheating due to difficulty in controlling the annealing temperature and an increase in energy cost occur in some cases.

The annealing temperature B is set in the temperature range from 620 °C to 740 °C. When the annealing temperature B is lower than 620 °C, the steel sheet is hard due to an incomplete recrystallization structure. Therefore, the yield strength of the steel sheet in the rolling direction is greater than 600 MPa, the cross-sectional hardness of the side portion of the crown cap after crown cap forming is greater than 220 Hv, the formability of the crown cap is poor, and the pressure resistance is low. However, when the annealing temperature B is higher than 740 °C, C derived from the carbide dissolved during annealing segregates and aggregates in the grain boundaries, the maximum grain size of the carbide in the cross section in the rolling direction after cooling is greater than 2.0 µm, the shapes of pleats become non-uniform in the formation of the crown cap, and the pressure resistance is decreased. Furthermore, during continuous annealing, threading problems such as heat buckling are likely to occur, which is undesirable. Thus, the annealing temperature B is set in the temperature range from 620 °C to 740 °C. In order to achieve both the formability and pressure resistance of the crown cap in a good balance, the annealing temperature B is preferably 640 °C or more. The annealing temperature B is preferably 720 °C or less.

In cooling in the annealing step, cooling is performed from the annealing temperature B to the cooling stop temperature C in the temperature range from 400 °C to 580 °C at an average cooling rate of 20 °C/s or more. When the average cooling rate is less than 20 °C/s, AlN precipitates excessively during cooling, the amount of N total-(N as AlN) is less than 0.0090%, the yield strength of the steel sheet in the rolling direction is less than 420 MPa, the cross-sectional hardness of the side portion of the crown cap after crown cap forming is less than 180 Hv, and the pressure resistance is low in some cases. Thus, the average cooling rate is set to 20 °C/s or more. The average cooling rate is preferably set to 40 °C/s or more. The upper limit of the average cooling rate is not particularly limited. When the average cooling rate is greater than 150 °C/s, the increase in strength of the steel sheet due to N total-(N as AlN) is saturated, the ductility is lowered due to the excessive precipitation of the carbide in ferrite grains, and cracking occurs in crown cap forming in some cases. Therefore, the average cooling rate is preferably 150 °C/s or less. The average cooling rate is more preferably 120 °C/s or less.

The cooling stop temperature C is set in the temperature range from 400 °C to 580 °C. When the cooling stop temperature is higher than 580 °C, AlN precipitates excessively, the amount of N total-(N as AlN) is less than 0.0090%, the yield strength of the steel sheet in the rolling direction is less than 420 MPa, the cross-sectional hardness of the side portion of the crown cap after crown cap forming is less than 180 Hv, and the pressure resistance is lowered in some cases. The cooling stop temperature is preferably set to 550 °C or less. The lower limit of the cooling stop temperature is set to 400 °C. When the cooling stop temperature is excessively low, the steel sheet is excessively hard, the shape formed becomes non-uniform in crown cap forming, and the pressure resistance is lowered in some cases. The cooling stop temperature is preferably set to 450 °C or more.

In a subsequent step after cooling at the above average cooling rate is stopped, the retention time in the temperature range from 400 °C to 580 °C is set to 30 seconds to 90 seconds. When the retention time in the temperature range from 400 °C to 580 °C is more than 90 seconds, the carbide grows due to C diffusion into the carbide in steel, the maximum grain size of the carbide in the cross section in the rolling direction is greater than 2.0 µm, the shapes of pleats become non-uniform in crown cap forming, and the pressure resistance is lowered. In order to ensure a good shape, the retention time in the temperature range from 400 °C to 580 °C is preferably set to 75 seconds or less. The lower limit of the retention time in the temperature range from 400 °C to 580 °C is set to 30 seconds or more. When the retention time is less than 30 seconds, the steel sheet is excessively hard, the shape becomes non-uniform in crown cap forming, and the pressure resistance is lowered.

The rolling reduction ratio during secondary cold rolling subsequent to the continuous annealing step is set to 1.0% to 12%. When the rolling reduction ratio during secondary cold rolling is less than 1.0%, the cross-sectional hardness of the side portion of the crown cap after crown cap forming is less than 180 Hv and the pressure resistance is lowered. The reason for this is unclear and is considered as described below. In steel sheets in which solute N is present, dislocations introduced by secondary cold rolling are anchored by solid solution during a heat treatment of lacquer baking. In the case when tension is applied subsequently, the anchored dislocations serve as barriers at deformation and the strength increases. On the other hand, in the case when crown caps are formed, drawing deformation is dominant and therefore force in slip systems which is different from tension acts. Therefore, the anchored dislocations do not act effectively during crown cap forming and the cross-sectional hardness of side portions of the crown caps is hard to increase. That is, in order to increase the cross-sectional hardness of the side portion of the crown cap in crown cap forming, a large number of dislocations need to be introduced by secondary cold rolling and the rolling reduction ratio needs to be 1.0% or more. When the rolling reduction ratio during secondary cold rolling is greater than 12%, dislocations are excessively introduced; hence, the cross-sectional hardness of the side portion of the crown cap is greater than 220 Hv, cracking occurs due to forming, and the pressure resistance is low. Thus, the rolling reduction ratio during secondary cold rolling is set to 1.0% to 12%. In order to achieve both the formability and pressure resistance of the crown cap, the rolling reduction ratio during secondary cold rolling is preferably 3.0% or more. The rolling reduction ratio during secondary cold rolling is preferably 10% or less.

A cold-rolled steel sheet obtained as described above is then subjected to a plating treatment such as tin plating, chromium plating, or nickel plating by, for example, electroplating as required such that a coated layer is formed on a surface of the steel sheet, whereby the steel sheet for crown caps is produced. The thickness of a film formed by surface treatment such as plating is sufficiently less than the thickness of the steel sheet and therefore the influence on mechanical properties of the steel sheet for crown caps is a negligible level.

As described above, the steel sheet for crown caps according to the present invention is capable of having sufficient strength and formability regardless of gauge reduction.

A crown cap according to the present invention is one which is formed by using the above-mentioned steel sheet for crown caps. The crown cap is mainly composed of a disk-shaped portion for covering the mouth of a bottle and a pleated portion placed therearound. The crown cap according to the present invention can be obtained in such a manner that a circular blank is stamped out, and formed by press forming. The crown cap according to the present invention is manufactured from the steel sheet for crown caps, the steel sheet having sufficient yield strength and excellent formability; is therefore excellent in pressure resistance as a crown cap regardless of gauge reduction; and has the effect of reducing the amount of waste discharged in association with use.

### EXAMPLES

In these examples, each of steels containing components shown in Table 1, the remainder being Fe and inevitable impurities, was produced in a converter and was continuously cast, whereby a steel slab was obtained. The obtained steel slab was reheated to 1,220 °C and was then subjected to hot rolling at a rolling start temperature of 1,150 °C and at a finish rolling temperature shown in Table 2, followed by coiling at a coiling temperature. Pickling was performed after hot rolling. Next, primary cold rolling was performed at a rolling reduction ratio shown in Table 2 and continuous annealing was performed under conditions shown in Table 2. Subsequently, secondary cold rolling was performed at a rolling reduction ratio shown in Table 2. An obtained steel sheet was continuously subjected to usual Cr plating, whereby tin-free steel was obtained.

**[Table 1]**

| (mass percent) | | | | | | | |
|---|---|---|---|---|---|---|---|
| Steel No. | C | Si | Mn | P | S | Al | N |
| A | 0.033 | 0.01 | 0.43 | 0.012 | 0.011 | 0.036 | 0.0147 |
| B | 0.046 | 0.01 | 0.21 | 0.014 | 0.010 | 0.033 | 0.0155 |
| C | 0.049 | 0.01 | 0.38 | 0.009 | 0.013 | 0.039 | 0.0138 |
| D | 0.041 | 0.01 | 0.46 | 0.013 | 0.014 | 0.058 | 0.0162 |
| E | 0.047 | 0.01 | 0.42 | 0.008 | 0.012 | 0.035 | 0.0106 |
| F | 0.043 | 0.01 | 0.44 | 0.015 | 0.011 | 0.032 | 0.0178 |
| G | 0.044 | 0.01 | 0.53 | 0.017 | 0.014 | 0.034 | 0.0146 |
| H | 0.022 | 0.01 | 0.49 | 0.018 | 0.013 | 0.038 | 0.0161 |
| I | 0.058 | 0.01 | 0.47 | 0.011 | 0.009 | 0.031 | 0.0144 |
| J | 0.077 | 0.01 | 0.36 | 0.010 | 0.011 | 0.029 | 0.0150 |
| K | 0.045 | 0.01 | 0.50 | 0.016 | 0.015 | 0.035 | 0.0137 |
| L | 0.051 | 0.01 | 0.38 | 0.013 | 0.017 | 0.056 | 0.0103 |
| M | 0.046 | 0.01 | 0.45 | 0.015 | 0.009 | 0.017 | 0.0176 |
| N | 0.024 | 0.01 | 0.53 | 0.014 | 0.015 | 0.057 | 0.0104 |
| O | 0.072 | 0.01 | 0.46 | 0.015 | 0.013 | 0.015 | 0.0175 |
| P | 0.013 | 0.01 | 0.43 | 0.016 | 0.011 | 0.036 | 0.0152 |
| Q | 0.096 | 0.01 | 0.46 | 0.010 | 0.016 | 0.028 | 0.0149 |
| R | 0.044 | 0.01 | 0.75 | 0.009 | 0.014 | 0.034 | 0.0141 |
| S | 0.039 | 0.01 | 0.51 | 0.012 | 0.012 | 0.078 | 0.0160 |
| T | 0.042 | 0.01 | 0.53 | 0.014 | 0.017 | 0.029 | 0.0084 |
| U | 0.038 | 0.01 | 0.39 | 0.013 | 0.011 | 0.036 | 0.0213 |
| V | 0.049 | 0.13 | 0.47 | 0.016 | 0.013 | 0.033 | 0.0156 |
| W | 0.051 | 0.01 | 0.48 | 0.034 | 0.015 | 0.035 | 0.0144 |

| | | | | | | | |
|---|---|---|---|---|---|---|---|
| Underlined portions: outside the scope of the present invention. | | | | | | | |

The steel sheet obtained as described above was subjected to a heat treatment corresponding to lacquer baking at 210 °C for 15 minutes, followed by tensile testing and measuring the cross-sectional hardness of a side portion of a crown cap. Tensile testing was performed using a tensile test specimen with a JIS #5 size in accordance with "JIS Z 2241", whereby the yield strength in a rolling direction was measured. For the cross-sectional hardness of the side portion of the crown cap, the steel sheet was formed into the crown cap, which was measured for Vickers hardness by a method according to "JIS Z 2244". For the crown cap, a circular blank with a diameter of 37 mm was used and the blank was formed to have dimensions (an outside diameter of 32.1 mm, a height of 6.5 mm, the number of pleats being 21) of a type-3 crown cap specified in "JIS S 9017" (abolished standard) by press forming. Evaluation positions were set to five points, in total, including one point at the center, two points in an upper surface direction of the crown cap, and two points in a downward direction of the crown cap as centered on a position (H/2) corresponding to half the height H of the crown cap. The Vickers indentation load was set to 100 gf and the intervals between the points were set to 3d (d: the length of a diagonal of an indentation). The average of the Vickers hardness values of the five points was defined as the cross-sectional hardness of the side portion of the crown cap.

For the grain size of a carbide in a cross section in the rolling direction, a through-thickness cross section parallel to the rolling direction of the steel sheet was polished and was then etched with an etchant (3 volume percent nital), a through-thickness one-fourth position (in the above cross section, a one-fourth position from a surface in a thickness direction) was observed over 10 fields of view at 2,000x magnification using a scanning electron microscope (SEM), and cementite was identified by visual judgment using a microstructure photograph taken with the SEM. For the size of cementite grains, the area of each cementite grain was determined by image analysis and was converted into the equivalent circle diameter, which was defined as the size of the cementite grain. The size of a cementite grain which was largest in size in the 10 fields of view was defined as the maximum grain size of the carbide in the cross section in the rolling direction.

The obtained steel sheet was used to form crown caps and was evaluated for crown cap formability. Circular blanks with a diameter of 37 mm were formed to have dimensions (an outside diameter of 32.1 mm, a height of 6.5 mm, the number of pleats being 21) of a type-3 crown cap specified in "JIS S 9017" (abolished standard) by press forming. For the evaluation of the formability of the crown caps, the length L of each fold 2 of the crown caps was measured as shown in Fig. 2, a crown cap in which the standard deviation of L-values was 0.1 or less was rated O, and a crown cap in which the standard deviation of L-values was greater than 0.1 was rated ×. The evaluation was performed for five of the crown caps. All the five crown caps in which the standard deviation of L-values was 0.1 or less were rated O (acceptable) and those other than these were rated × (unacceptable).

A pressure test was performed using the formed crown caps. A polyvinyl chloride liner was attached to the inside of the upper surface of each crown cap, a commercially available beer bottle was capped with the crown cap, a thin hole was made in an upper portion of the crown cap, a tool for feeding air into the bottle was fit therein, and the internal pressure of the bottle was increased by injecting air into the bottle at a rate of 5 psi per second. Conditions for increasing the pressure in the bottle are as follows: the pressure in the bottle was increased to 100 psi (a pressurizing operation), was held at 100 psi for 1 minute (a holding operation), and was increased again at 5 psi per second (a repressurizing operation). In each of the pressurizing operation, the holding operation, and the repressurizing operation, the internal pressure of the bottle that was obtained when air leaked from a gap between the crown cap and the mouth of the bottle or when the crown cap was detached from the bottle mouth (decapping) was defined as the pressure resistance value of the crown cap. The case where an anti-pressure value equal to or greater than that of a conventional crown cap was exhibited was rated O. The case where the anti-pressure value of the conventional crown cap was not exhibited was rated ×. After a rating of × was assigned, further evaluation was difficult; hence, - was given in the following tables. Incidentally, the conventional crown cap used was made from an SR (single reduced) steel sheet with a thickness of 0.22 mm. The case where a rating of O was obtained in all of the pressurizing operation, the holding operation, and the repressurizing operation was excellent in pressure resistance and was comprehensively rated O (acceptable). The case other than that was poor in pressure resistance and was rated × (unacceptable). Obtained results are shown in Table 2.

As is clear from Table 2, steel sheets of Steel Sheet Nos. 1 to 15 that were inventive examples had components within the scope of the present invention, had a yield strength of 420 MPa to 600 MPa in a rolling direction, and had the maximum grain size of a carbide 2.0 µm or less in a cross section in a rolling direction. A crown cap formed from each of Steel Sheet Nos. 1 to 15 was such that the cross-sectional hardness of a side portion of the crown cap after crown cap forming was 180 Hv to 220 Hv. Steel sheets for crown caps of Steel Sheet Nos. 1 to 15 were good in both crown cap formability and pressure resistance.

On the other hand, it was clear that a steel sheet of Steel Sheet No. 16 that was a comparative example was such that since the content of C was less than 0.02%, the yield strength of the steel sheet in the rolling direction thereof was less than 420 MPa, the cross-sectional hardness of a side portion of a crown cap after crown cap forming was less than 180 Hv, the crown cap formability was good, but the pressure resistance was insufficient.

It was clear that a steel sheet of Steel Sheet No. 17 was such that since the content of C was greater than 0.08%, the yield strength of the steel sheet in the rolling direction thereof was greater than 600 MPa, the maximum grain size of a carbide in a cross section in a rolling direction was greater than 2.0 µm, and the cross-sectional hardness of a side portion of a crown cap after crown cap forming was greater than 220 Hv; and therefore, the crown cap formability was poor, and the pressure resistance was insufficient.

It was clear that a steel sheet of Steel Sheet No. 18 was such that since the content of Mn was greater than 0.60%; the yield strength in a rolling direction was greater than 600 MPa, and the cross-sectional hardness of a side portion of a crown cap after crown cap forming was greater than 220 Hv; and therefore, the shapes of pleats of the formed crown cap were non-uniform, and shape failures occurred to cause a reduction in pressure resistance.

It was clear that a steel sheet of Steel Sheet No. 19 was such that since the content of Al was greater than 0.06%; N total-(N as AlN) was less than 0.0090%, the yield strength of the steel sheet in the rolling direction thereof was less than 420 MPa, and the cross-sectional hardness of a side portion of a crown cap after crown cap forming was less than 180 Hv; and therefore the pressure resistance was insufficient.

It was clear that a steel sheet of Steel Sheet No. 20 was such that since the content of N was less than 0.0100%, N total-(N as AlN) was less than 0.0090%; the yield strength of the steel sheet in the rolling direction thereof was less than 420 MPa, and the cross-sectional hardness of a side portion of a crown cap after crown cap forming was less than 180 Hv; and therefore the pressure resistance was insufficient.

It was clear that a steel sheet of Steel Sheet No. 21 was such that since the content of N was greater than 0.0180%, N total-(N as AlN) was greater than 0.0170%; the yield strength of the steel sheet in the rolling direction thereof was greater than 600 MPa, and the cross-sectional hardness of a side portion of a crown cap after crown cap forming was greater than 220 Hv; and therefore the formed crown cap was poor in shape, and the pressure resistance was insufficient.

It was clear that since the content of Si in a steel sheet of Steel Sheet No. 22 was greater than 0.02% and the content of P in a steel sheet of Steel Sheet No. 23 was greater than 0.020%; each of the steel sheets of Steel Sheet No. 22 and the steel sheet of Steel Sheet No. 23 was such that the yield strength in the rolling direction was greater than 600 MPa, and the cross-sectional hardness of a side portion of a crown cap after crown cap forming was greater than 220 Hv; and therefore shape failures occurred, and the pressure resistance was insufficient.

Next, each of steels containing components of Steel Nos. B, G, K, and S shown in Table 1, the remainder being Fe and inevitable impurities, was produced in a converter and was continuously cast, whereby a steel slab was obtained. Manufacturing conditions shown in Table 3 were applied to the obtained steel slab. An obtained steel sheet was continuously subjected to usual Cr plating, whereby tin-free steel was obtained. Steel Sheet Nos. 24 to 56 obtained as described above were subjected to a heat treatment corresponding to paint baking at 210 °C for 15 minutes, followed by determining the yield strength in a rolling direction, the maximum grain size of a carbide in a cross section in the rolling direction, and the cross-sectional hardness of a side portion of a crown cap after crown cap forming by the above-mentioned methods. Furthermore, the crown cap formability and the pressure resistance were evaluated by the above-mentioned methods.

As is clear from Table 3, steel sheets of Steel Sheet Nos. 27, 28, 30, 32, 33, 35, 37 to 39, 41, 42, 45 to 48, and 50 to 52 that were inventive examples were such that the maximum grain size of a carbide in a cross section in a rolling direction was 2.0 µm or less, the yield strength in the rolling direction was 420 MPa to 600 MPa, the cross-sectional hardness of a side portion of a crown cap after crown cap forming was 180 Hv to 220 Hv, and therefore the crown cap formability and the pressure resistance were both good.

On the other hand, it was clear that a steel sheet of Steel Sheet No. 24 that was a comparative example was such that since the coiling temperature was higher than 670 °C, the amount of N total-(N as AlN) was less than 0.0090%; the yield strength of the steel sheet in the rolling direction was less than 420 MPa, the cross-sectional hardness of a side portion of a crown cap after crown cap forming was less than 180 Hv, and the maximum grain size of a carbide in a cross section in a rolling direction was greater than 2.0 µm; and therefore the shapes of pleats of the crown cap became non-uniform during crown cap forming, shape failures occurred, the crown cap formability was poor, and the pressure resistance was poor.

It was clear that a steel sheet of Steel Sheet No. 25 was such that since the average heating rate in a temperature range A from 500 °C to 600 °C was less than 10 °C/s, the amount of N total-(N as AlN) was less than 0.0090%, the yield strength of the steel sheet in the rolling direction thereof was less than 420 MPa, the cross-sectional hardness of a side portion of a crown cap after crown cap forming was less than 180 Hv, and the pressure resistance was poor.

It was clear that a steel sheet of Steel Sheet No. 26 was such that since the annealing temperature was lower than 620 °C, the steel sheet was hard due to an incomplete recrystallization structure; the yield strength of the steel sheet in the rolling direction thereof was greater than 600 MPa, and the cross-sectional hardness of a side portion of a crown cap after crown cap forming was greater than 220 Hv; and the crown cap formability was poor, and the pressure resistance was poor.

It was clear that a steel sheet of Steel Sheet No. 29 was such that since the annealing temperature was higher than 740 °C, the maximum grain size of a carbide in a cross section in a rolling direction was greater than 2.0 µm, the shapes of pleats became non-uniform in the formation of a crown cap, and the pressure resistance was poor.

It was clear that a steel sheet of Steel Sheet No. 31 was such that since the average heating rate in a temperature range A from 500 °C to 600 °C was greater than 30 °C/s, the steel sheet was hard; the yield strength of the steel sheet in the rolling direction thereof was greater than 600 MPa, and the cross-sectional hardness of a side portion of a crown cap after crown cap forming was greater than 220 Hv; and the crown cap formability was poor, and the pressure resistance was poor.

It was clear that a steel sheet of Steel Sheet No. 34 was such that since the average cooling rate was less than 20 °C/s although the cooling stop temperature C was in a temperature range from 400 °C to 580 °C, the amount of N total-(N as AlN) was less than 0.0090%; the yield strength of the steel sheet in the rolling direction thereof was less than 420 MPa, and the cross-sectional hardness of a side portion of a crown cap after crown cap forming was less than 180 Hv; and the pressure resistance was poor.

It was clear that a steel sheet of Steel Sheet No. 36 was such that since the cooling stop temperature was higher than 580 °C, the amount of N total-(N as AlN) was less than 0.0090%; the yield strength of the steel sheet in the rolling direction thereof was less than 420 MPa, and the cross-sectional hardness of a side portion of a crown cap after crown cap forming was less than 180 Hv; and the pressure resistance was poor.

It was clear that a steel sheet of Steel Sheet No. 40 was such that since the cooling stop temperature was lower than 400 °C, the steel sheet was hard; the yield strength of the steel sheet in the rolling direction thereof was greater than 600 MPa, and the cross-sectional hardness of a side portion of a crown cap after crown cap forming was greater than 220 Hv; the crown cap formability was poor, and the pressure resistance was poor. Incidentally, in Table 3, the retention time of each of the steel sheets of Steel Sheet Nos. 36 and 40 in a temperature range from 400 °C to 580 °C represents the retention time at the cooling stop temperature C.

It was clear that steel sheets of Steel Sheet Nos. 43 and 53 were such that since the rolling reduction ratio during secondary cold rolling was greater than 12%, the yield strength of the steel sheets in the rolling direction thereof was greater than 600 MPa, and the cross-sectional hardness of a side portion of a crown cap after crown cap forming was greater than 220 Hv; the crown cap formability was poor, and the pressure resistance was poor.

It was clear that a steel sheet of Steel Sheet No. 44 was such that since the rolling reduction ratio during secondary cold rolling was less than 1.0%, the yield strength of the steel sheet in the rolling direction thereof was less than 420 MPa, the cross-sectional hardness of a side portion of a crown cap after crown cap forming was less than 180 Hv, and the pressure resistance was low.

It was clear that a steel sheet of Steel Sheet No. 49 was such that since the retention time in a temperature range from 400 °C to 580 °C was more than 90 seconds although the cooling stop temperature C was in the temperature range from 400 °C to 580 °C, the maximum grain size of a carbide in a cross section in a rolling direction was greater than 2.0 µm; the shapes of pleats became non-uniform during crown cap forming, and the pressure resistance was poor.

It was clear that a steel sheet of Steel Sheet No. 54 was such that since the retention time in a temperature range from 400 °C to 580 °C was less than 30 seconds although the cooling stop temperature C was in the temperature range from 400 °C to 580 °C, the steel sheet was hard, the yield strength of the steel sheet in the rolling direction thereof was greater than 600 MPa, the cross-sectional hardness of a side portion of a crown cap after crown cap forming was greater than 220 Hv; the crown cap formability was poor, and the pressure resistance was poor.

It was clear that steel sheets of Steel Sheet Nos. 55 and 56 were such that since the content of Al was greater than 0.06%, N total-(N as AlN) was less than 0.0090%; the yield strength of the steel sheets in the rolling direction was less than 420 MPa, and the cross-sectional hardness of a side portion of a crown cap after crown cap forming was less than 180 Hv; and the pressure resistance was poor. Reference Signs List

- 1: Upper surface of crown cap
- 2: pleats

## Claims

1. A cold-rolled steel sheet for crown caps, having a composition containing
C: 0.02% to 0.08%,
Si: 0.02% or less,
Mn: 0.10% to 0.60%,
P: 0.020% or less,
S: 0.020% or less,
Al: 0.01% to 0.06%, and
N: 0.0100% to 0.0180%
on a mass basis, the remainder being Fe and inevitable impurities,
wherein N total-(N as AlN) is 0.0090% to 0.0170%,
the maximum grain size of a carbide is 0.3 µm or more and 2.0 µm or less in a cross section in a rolling direction, measured according to the description, and
the yield strength, measured using a tensile test specimen with a JIS #5 size in accordance with "JIS Z 2241" and after a heat treatment at 210° C for 15 minutes, is 420 MPa to 600 MPa in the rolling direction,
where the N total is the total amount of N and the N as AlN is the amount of N present in the form of AlN, the N present in AlN being confirmed by dissolving and extracting AlN by a 10% Br-methanol solution and N present in the AlN quantitatively analyzed by absorptiometry.

2. A method for manufacturing a steel sheet for crown caps, comprising:
a hot rolling step of performing coiling at a temperature of 670 °C or less after finish rolling in the hot rolling of a steel material having the composition specified in Claim 1;
a primary cold rolling step of performing cold rolling after the hot rolling step;
a continuous annealing step of performing heating at an average heating rate of 10 °C/s to 30 °C/s in a temperature range A from 500 °C to 600 °C in a heating course after the primary cold rolling step, annealing at a annealing temperature B in a temperature range from 620 °C to 740 °C,
cooling from the annealing temperature B to a cooling stop temperature C in a temperature range from 400 °C to 580 °C at an average cooling rate of 20 °C/s or more, and retaining in the temperature range from 400 °C to 580 °C for a retention time of 30 seconds to 90 seconds after cooling at the above average cooling rate is stopped; and
a secondary cold rolling step of performing cold rolling at a rolling reduction ratio of 1.0% to 12% after the continuous annealing step.

3. A crown cap formed by using the steel sheet for crown caps according to Claim 1.

4. The crown cap according to Claim 3, wherein the cross-sectional hardness of a side portion of the crown cap is 180 Hv to 220 Hv.

## Patentansprüche

1. Kaltgewalztes Stahlblech für Kronkorken, das eine Zusammensetzung hat, die Folgendes enthält:
C: 0,02 % bis 0,08 %,
Si: 0,02% oder weniger,
Mn: 0,10% bis 0,60 %,
P: 0,020 % oder weniger,
S: 0,020 % oder weniger,
Al: 0,01 % bis 0,06 %, und
N: 0,0100 % bis 0,0180 %
auf die Masse bezogen, der Rest ist Fe und unvermeidbare Verunreinigungen,
worin N insgesamt (N als AlN) 0,0090 % bis 0,0170 % beträgt, die maximale Korngröße eines Carbids 0,3 µm oder
mehr und 2,0 µm oder weniger in einem Querschnitt in einer Walzrichtung beträgt, gemessen entsprechend der Beschreibung, und
die Streckgrenze, gemessen an einer Zugfestigkeitsprobe mit einer Größe von JIS #5 entsprechend "JIS Z 2241" und nach einer 15-minütigen Erwärmung bei 210 °C, beträgt 420 MPa bis 600 MPa in Walzrichtung,
wobei die N-Gesamtmenge die Gesamtmenge von N und das N als AlN die in Form von AlN vorhandene Menge von N ist, wobei das in AlN vorhandene N durch Auflösen und Extrahieren von AlN durch eine 10 %ige Br-Methanollösung bestätigt wird und
das in AlN vorhandene N quantitativ durch Absorptionsmessung analysiert wird.

2. Verfahren zur Herstellung eines Stahlblechs für Kronkorken, umfassend:
einen Warmwalzschritt zur Durchführung des Wickelns bei einer Temperatur von 670 °C oder weniger nach dem Fertigwalzen beim Warmwalzen eines Stahlmaterials mit einer Zusammensetzung nach Anspruch 1; einen primären Kaltwalzschritt zur Durchführung des Kaltwalzens nach dem Warmwalzschritt;
einen kontinuierlichen Glühschritt, bei dem nach dem primären Kaltwalzschritt ein Erwärmen mit einer durchschnittlichen Aufheizrate von 10 °C/s bis 30 °C/s in einem Temperaturbereich A von 500 °C bis 600 °C in einem Erwärmungsverlauf durchgeführt wird, Glühen bei einer Glühtemperatur B in einem Temperaturbereich von 620 °C bis 740 °C, Abkühlen von der Glühtemperatur B auf eine Kühlstopptemperatur C in einem Temperaturbereich von 400 °C bis 580 °C mit einer durchschnittlichen Abkühlgeschwindigkeit von 20 °C/s oder mehr und Halten im Temperaturbereich von 400 °C bis 580 °C für eine Verweilzeit von 30 Sekunden bis 90 Sekunden, nachdem die Abkühlung mit der oben genannten durchschnittlichen Abkühlgeschwindigkeit gestoppt wurde; und
einen sekundären Kaltwalzschritt zur Durchführung des Kaltwalzens mit einem Walzreduktionsverhältnis von 1,0 % bis 12 % nach dem kontinuierlichen Glühen.

3. Kronkorken, der unter Verwendung des Stahlblechs für Kronkorken entsprechend Anspruch 1 geformt wurde.

4. Kronkorken nach Anspruch 3, wobei die Querschnittshärte eines Seitenteils des Kronkorkens 180 Hv bis 220 Hv beträgt.

## Revendications

1. Tôle d'acier laminée à froid pour capsule-couronnes, ayant une composition contenant
C : de 0,02 % à 0,08 %,
Si : 0,02 % ou moins,
Mn : de 0,10 % à 0,60 %,
P : 0,020 % ou moins,
S : 0,020 % ou moins,
Al : de 0,01 % à 0,06 %, et
N : de 0,0100 % à 0,0180 %
sur une base massique, le reste étant du Fe et des impuretés inévitable,
où total de N - (N comme AlN) est de 0,0090 % à 0,0170 %,
la taille de grain maximum d'un carbure est de 0,3 µm ou plus et de 2,0 µm ou moins dans une section transversale dans une direction de laminage, mesurée conformément à la description, et
la limite d'élasticité, mesurée à l'aide d'un spécimen de test de traction de taille JIS #5 selon « JIS Z 2241 » et après un traitement thermique à 210°C pendant 15 minutes, est de 420 MPa à 600 MPa dans la direction du laminage,
dans laquelle le total de N est la quantité totale de N et le N comme AlN est la quantité de N présent sous forme de AlN, le N présent dans AlN étant confirmé par dissolution et extraction de AlN par une solution de Br-méthanol à 10 % et le N présent dans l'AlN analysé quantitativement par absorptiométrie.

2. Procédé de production d'une tôle d'acier pour capsule-couronne, comprenant :
une étape de laminage à chaud consistant à effectuer un bobinage à une température de 670°C ou moins après un laminage de finition dans le laminage à chaud d'un matériau d'acier ayant la composition spécifiée dans la revendication 1 ;
une étape de laminage à froid primaire consistant à effectuer un laminage à froid après l'étape de laminage à chaud ;
une étape de recuit continu consistant à effectuer un chauffage à une vitesse de chauffage moyenne de 10°C/s à 30°C/s dans une plage de température A de 500°C à 600°C dans un processus de chauffage après l'étape de laminage à froid primaire, un recuit à une température de recuit B dans une plage de température de 620°C à 740°C, un refroidissement à partir de la température de recuit B à une température d'arrêt de refroidissement C dans une plage de température de 400°C à 580°C à une vitesse de refroidissement moyenne de 20°C/s ou plus, et une rétention dans la plage de température de 400°C à 580°C pendant un temps de rétention de 30 secondes à 90 secondes après l'arrêt du refroidissement à la vitesse de refroidissement moyenne ci-dessus ; et
une étape de laminage à froid secondaire consistant à effectuer un laminage à froid à un taux de réduction de laminage de 1,0 % à 12 % après l'étape de recuit continu.

3. Capsule-couronne formée en utilisant la tôle d'acier pour capsules-couronnes selon la revendication 1.

4. Capsule-couronne selon la revendication 3, dans laquelle la dureté de section transversale d'une partie latérale de la capsule-couronne est de 180 Hv à 220 Hv.
